

Nov. 10, 1936.

R. P. HEUER

2,060,073

## COPPER REFINING METHOD

Filed June 5, 1930

2 Sheets-Sheet 1

Witnesses:  
T. H. Fonda,  
Walter Chinn

*By*

W. Steel Johnson

INVENTOR  
Russell P. Heuer,

Attorney.



Nov. 10, 1936.

R. P. HEUER

2,060,073

## COPPER REFINING METHOD

Filed June 5, 1930

2 Sheets-Sheet 2



*Witnesses*

W. C. Fonda

Walter Chinn

By

Inventor  
Russell P. Heuer,  
y  
John Steele Jackson  
Attorney.

## UNITED STATES PATENT OFFICE

2,060,073

## COPPER REFINING METHOD

Russell P. Heue, Haverford, Pa., assignor to The American Metal Company Limited, New York, N. Y., a corporation of New York

Application June 5, 1930, Serial No. 459,300

37 Claims. (Cl. 75—10)

My invention relates to methods for refining copper. The apparatus shown herein is claimed in my application, Serial Number 605,389, filed April 15, 1932, for copper refining apparatus.

5 A purpose of my invention is to produce commercial copper substantially free from cuprous oxide and at the same time having so few gas cavities as not to interfere with the mechanical working of the copper.

10 A further purpose is to reduce by means of carbon the content of copper oxide to a point much below that reached under the present practice.

A further purpose is to crowd carbon into the body of a substantially sulphur-free copper melt 15 in order to reduce the cuprous oxide content to a minimum.

A further purpose is to roast solid copper cathodes to substantially eliminate the sulphur, melt the cathodes, and reduce any cuprous oxide 20 present in the molten copper by contact with carbon, avoiding blowing and poling, and obtaining an oxide-free copper having no dissolved gaseous impurities except carbon monoxide.

A further purpose is to eliminate sulphur contamination from solid copper by reduction with 25 hydrogen, remove any dissolved hydrogen by melting in an oxidizing atmosphere and cast the resulting copper.

A further purpose is to obtain commercial 30 copper castings free from any excess of carbon dioxide, water vapor or hydrogen, and consequently without gas cavities due to the liberation of these impurities during the solidification period of the copper.

35 A further purpose is to deoxidize copper beyond the point at which it is microscopically oxygen free so that it can be solidified into castings substantially free from gas cavities and to cast the copper preferably while protecting it from the atmosphere, desirably by carbon monoxide free from contaminating gases.

Further purposes will appear in the specification and in the claims.

In the drawings, Figure 1 is a top plan view of 45 an arrangement of furnaces by which my methods may be desirably performed.

Figure 2 is an enlarged vertical section of the carbon reducing furnace seen in Figure 1.

50 Figures 3 to 5 are diagrammatic views useful in explaining my invention.

In the drawings like numerals refer to like parts.

The common practice is to melt copper cathodes in large intermittent reverberatory furnaces. 55 In such furnaces, the conventional mode of oper-

ation is as follows: (1) charging; (2) melting; (3) blowing; (4) skimming; (5) poling; (6) casting. The process introduces many impurities into the metal which seriously impair the grade of the products.

Copper cathodes commonly carry copper sulphate on the surface, or occluded between copper crystals. This sulphur, as well as sulphur from the gases of combustion, forms as an impurity in the molten copper. Oxygen is also present in the bath as dissolved cuprous oxide. The blowing, while removing part of the sulphur, increases the oxygen content of the bath and saturates the bath with nitrogen and other gases from the atmosphere.

The primary purpose of the poling operation is to remove the excess of oxygen, present largely in the form of cuprous oxide. In doing so, however, the bath takes up hydrogen, carbon monoxide, carbon dioxide and water vapor from the organic matter.

At times during the poling operation the bath is protected by charcoal or coke floating upon the surface. By virtue of its position and its small quantity as compared with the bath, the amount of reduction possible from carbon used in this manner is negligible.

Previous observers have noticed that, when the poling operation is carried too far, the copper is valueless because of the large numbers of gas 30 cavities. As stated by H. O. Hofman (Metallurgy of Copper, McGraw-Hill Book Co., Inc., New York, 1914, page 384): "It is important that some Cu<sub>2</sub>O remain in the copper, as the dissolving power of copper for gas is greatly weakened by 35 its presence." The general feeling has been that in some way the presence of Cu<sub>2</sub>O decreases the solubility of the copper for gases, and consequently avoids the danger of gas cavities. Another explanation which has been put forward is that the 40 copper would become more highly saturated with reducing gases as poling proceeded farther, and the solubility of the copper for the gases would decrease on cooling, causing them to separate as 45 gas cavities during solidification. It is commonly considered bad practice to reduce the content of Cu<sub>2</sub>O below 0.3%.

From physical-chemical studies of the poling operation I have discovered that the commonly accepted explanations of the role of cuprous oxide are incorrect, and that the retention of cuprous oxide in the copper is undesirable and unnecessary. What has been attributed to solubility is really due to reactions which occur whenever cuprous oxide is present.

The reduction of cuprous oxide under the conditions of poling takes place according to the following reactions:



I will consider the above reactions in terms of the thermodynamic activities of the reacting components and of the standard free energy changes for each reaction where the activities of the reacting components are referred to arbitrarily chosen standard states for the reacting components in which their activities are unity. (See Gilbert Newton Lewis and Merle Randall, Thermodynamics and Free Energy of Chemical Substances, McGraw-Hill Book Co., Inc., New York, first edition, 1923, chapters XXII and XXIV, and pages 190, 255, and 293.)

15 Thus for the reaction



the relationship between the activities and the standard free energy change would be as follows:

$$25 \quad -\Delta F_0 = RT \ln \frac{(A.Y)(A.Z)}{(A.W)(A.X)} \quad (5)$$

$\Delta F_0$  = standard free energy change  
 $R$  = gas constant  
 $T$  = absolute temperature  
 $(A.W)$  = activity of component  $W$   
 $(A.X)$  = activity of component  $X$   
 $(A.Y)$  = activity of component  $Y$   
 $(A.Z)$  = activity of component  $Z$

35 Since at constant temperature the logarithm becomes constant, the expression of Equation (5) is frequently simplified under the name of the law of "mass action". When this is done, the pressures of gases and the molalities of dilute solutions are ordinarily substituted for the activities.

40 Applying Equation (5) to Reaction (1), and using the same nomenclature, we get:

$$45 \quad -\Delta F_0 = RT \ln \frac{(A.\text{Cu})^2(A.\text{CO})}{(A.\text{Cu}_2\text{O})(A.\text{C})} \quad (6)$$

$(A.\text{Cu})$  = activity of copper  
 $(A.\text{CO})$  = activity of carbon monoxide  
 $(A.\text{Cu}_2\text{O})$  = activity of cuprous oxide  
 $(A.\text{C})$  = activity of carbon

in the above reaction equilibrium is never reached during poling. It is only attained when the cuprous oxide is practically all removed.

55 Applying the general form of Equation (5) to Reaction (2), and using the previous nomenclature, we obtain:

$$60 \quad -\Delta F_0 = RT \ln \frac{(A.\text{Cu})^2(A.\text{CO}_2)}{(A.\text{Cu}_2\text{O})(A.\text{CO})} \quad (7)$$

$(A.\text{CO}_2)$  = activity of carbon dioxide

It is probable that the bath will become saturated with carbon dioxide during the poling operation, so that  $(A.\text{CO}_2)$  will be constant. Also,  $(A.\text{Cu})$  is constant as the bath is practically pure copper.

65 Then Equation (7) becomes:

$$60 \quad -\Delta F_0 = RT \ln \frac{K}{(A.\text{Cu}_2\text{O})(A.\text{CO})} \quad (8)$$

70 where  $K$  is a constant for the particular conditions. At constant temperature this expression becomes:

$$(A.\text{Cu}_2\text{O})(A.\text{CO}) = K_1 \quad (9)$$

75  $K_1$  = proper constant

Equation (9) has been plotted in Figure 3, using  $(A.\text{Cu}_2\text{O})$  values as the abscissae and  $(A.\text{CO})$  values as the ordinates.

Using the same symbols, the expression for Reaction (3) is:

$$70 \quad -\Delta F_0 = RT \ln \frac{(A.\text{Cu})^2(A.\text{H}_2\text{O})}{(A.\text{Cu}_2\text{O})(A.\text{H}_2)} \quad (10)$$

$(A.\text{H}_2\text{O})$  = activity of water

$(A.\text{H}_2)$  = activity of hydrogen

10 Since the activities of copper and of water are constant, this equation becomes, at constant temperature:

$$15 \quad (A.\text{Cu}_2\text{O})(A.\text{H}_2) = K_2 \quad (11)$$

$K_2$  = proper constant

Equation (11) has been plotted in Figure 4, using  $(A.\text{Cu}_2\text{O})$  values as the abscissae and  $(A.\text{H}_2)$  values as the ordinates.

20 The activity of any component is a function of the concentration. Therefore, we may observe the relation between the concentration of carbon monoxide or hydrogen and that of the cuprous oxide by the use of the curves shown in Figures 25 3 and 4.

For example, with a high cuprous oxide concentration, corresponding to the point  $a$ , the concentrations of hydrogen and carbon monoxide are low. As the concentration of cuprous oxide falls, as shown progressively at points  $b$ ,  $c$ , and  $d$ , the concentrations of hydrogen and carbon monoxide remain substantially the same.

25 When the cuprous oxide content reaches a low enough value, as that indicated by  $e$  or  $f$ , at the knees of the curves, the concentrations of hydrogen and carbon monoxide rise. When the concentration of cuprous oxide is reduced progressively below that represented by the point  $f$ , a rapid rise in concentration of hydrogen or carbon monoxide occurs, entirely out of proportion to the decrease in the concentration of cuprous oxide.

30 In the practical operation of the refining furnace, poling is stopped at about the point  $g$  on the respective curves of Figures 3 and 4, representing a cuprous oxide content of about 0.3%. Previous observers have considered that it is necessary to stop at this point, either because the cuprous oxide reduces the solubility of gases in the copper, as suggested by Hofman, or because the copper will become more highly saturated with reducing gases as the poling proceeds further, and these reducing gases will separate out on cooling. Both of these explanations have been 40 found by me to be erroneous.

35 As previously stated, it is not the separation of carbon monoxide and hydrogen because of lower solubility in solid than in liquid copper, or because of any other reason, which causes the bulk of the gas cavities, but rather the reactions during solidification of the dissolved carbon monoxide and hydrogen with any remaining cuprous oxide to produce carbon dioxide and water vapor with which copper has been saturated already.

45 By reference to Reactions (1), (2) and (3) it will be seen that Reaction (1) can hardly take place during the solidification of the casting, because no carbon is present at that time. However, Reactions (2) and (3) could occur, since both carbon monoxide and hydrogen are present in copper made by the prior art commercial process.

50 During the solidification of copper containing less than 3.45% of cuprous oxide, crystals of pure 75

copper will first separate out, thus concentrating the cuprous oxide in the supernatant liquid along the line DE as shown in the conventional temperature-composition curve for the system cuprous oxide-copper, reproduced in Figure 5. (See Hofman, Metallurgy of Copper, McGraw-Hill Book Co., Inc., New York, 1914, page 13.)

At the eutectic temperature (E in Figure 5), 1065° C., the liquid will contain 3.45% of cuprous oxide. This increase in the concentration of cuprous oxide during solidification causes the Reactions (2) and/or (3) to proceed rapidly, yielding carbon dioxide and/or water vapor.

Thus it will be seen that overpoling and excessive gas cavities are due just as much to the presence of cuprous oxide in the copper as they are to the presence of reducing gases, such as hydrogen and carbon monoxide. I propose therefore to eliminate cuprous oxide, thus avoiding the injury done to the copper from overpoling and excessive gas release, and by producing copper free from cuprous oxide, I obtain better physical properties and higher electrical conductivity in the product.

The solubility of hydrogen in molten copper is considerably greater than its solubility in solid copper at the freezing temperature. On the other hand, there is substantially no change in the solubility of carbon monoxide when copper solidifies. Therefore, forgetting for the moment the question of reactions with cuprous oxide, carbon monoxide is a much less undesirable ingredient in molten copper than hydrogen. I avoid the presence of excessive quantities of hydrogen or remove it before casting, whether or not cuprous oxide is present. Carbon monoxide, however, is not particularly harmful from the standpoint of change of solubility on solidification, nor of formation by any reaction possible during solidification, so that I may even saturate the bath with carbon monoxide as later explained.

Poling is necessitated by blowing, and blowing is required in order to remove sulphur. To eliminate both blowing and poling I propose to eliminate sulphur from the cathodes prior to melting them, rather than to attempt to oxidize sulphur out of the molten bath. Having eliminated sulphur, I melt the cathodes under conditions which prevent any absorption of sulphur.

My low sulphur bath does not require blowing, and therefore does not have the high oxygen content due to blowing, and the saturation with other atmospheric gases for which it is responsible. The elimination of poling enables me to avoid the attendant contamination with hydrogen, carbon dioxide and water vapor.

Hydrogen, carbon dioxide and water vapor tend to produce gas as previously explained, but carbon monoxide does not of itself act in this way because it is not formed by any of the reactions which occur during cooling, and its solubility does not greatly decrease when the copper solidifies.

As a further precaution against the possibility of reactions occurring between hydrogen or carbon monoxide and cuprous oxide during cooling, I reduce the cuprous oxide in the resultant metal much below any content which has been deemed possible heretofore. The reduction of cuprous oxide until only a trace is present is best performed by a large exposed surface of solid carbon in contact with the bath.

In the drawings I show apparatus suitable for carrying out my methods, but do intend to indicate that this is by any means the only ap-

paratus which might be employed. The roasting or calcining operation to remove sulphur is best performed in the continuous flue of a furnace as shown in my Patent, No. 1,914,716, for Copper melting furnace, granted June 20, 1933, or in Lukens and Heuer Patent, No. 1,733,419, for Continuous copper melting furnace, granted October 29, 1928.

It will be understood, however, that my invention is not restricted to use with a continuous furnace.

The furnace A of Figure 1 is of the general type shown in my Patent, No. 1,914,716, above referred to. Cold cathodes are charged at 8 by any suitable pusher 10 on to the continuous hearth 11 operating in the flue 12. The hearth is moved by a motor 13 and any suitable connections. In the illustration shown the piles of cathodes 14 are carried clockwise to the discharge point 15, where they are picked up by the fork 16 and carried into the furnace 17 and there dropped. The charging fork 16 is desirably moved in and out through a door 18.

In the furnace 17, the bath 19, desirably covered by a suitable protective slag, is heated by products of combustion from burners at 20. I prefer to use oil burners, but it will be understood that any suitable means of heating may be employed. From the furnace 17 the products of combustion pass through the neck 21, through which the cathodes are charged, and around the flue in a counter-clockwise direction, finally rising through the stack 22. During normal operation of the furnace, the products of combustion are prevented from taking a clockwise path by the wall 23.

The hearth 11 in the flue 12 may be continuous or may consist of a plurality of cars separately moved about the flue. The continuous mode of operation is much superior, and therefore I indicate the hearth as extending around the flue and being turned by any suitable driving means 13.

The preheating and roasting chamber 12 contains a non-reducing atmosphere. The copper sulphate or other sulphur compound adhering to the cathode is calcined, and is decomposed by the products of combustion. The sulphur is carried off as sulphur dioxide.

During roasting, the cathodes should be heated to about 815° C. to complete the formation of sulphur dioxide. Lower temperatures will suffice, although operation is slower in that case. Higher temperatures will work satisfactorily provided care is taken not to melt the cathodes in the flue. Melting here is objectionable for various reasons, metallurgically because molten copper will dissolve the copper oxide and copper sulphide formed, reducing the thermodynamic activity and preventing a quantitative elimination of sulphur.

While I consider the method of desulphurizing as carried out in a roasting or calcining flue to be preferable, I may also desulphurize solid copper in furnaces free from combustion gases, as, for example, muffles or electric furnaces. In furnaces of this type, I may desulphurize by reducing with hydrogen, so that copper sulphate, copper sulphide and similar sulphur compounds will give up their sulphur in the form of hydrogen sulphide. Here also, the presence of molten copper is undesirable for the reason above stated.

Where reduction with hydrogen is employed, I will preferably melt the copper under slightly oxidizing furnace conditions to remove dissolved

hydrogen, which might otherwise produce gas cavities in the castings.

The preheating operation in a furnace of the type of furnace A should last about one hour, although the time taken by a given pile of cathodes in traversing the flue varies with the size of the furnace, and the type of cathode.

In order to melt the cathodes, I prefer to plunge them into a bath of molten copper, preferably suitably protected from contamination with sulphur from the flue gases by a suitable slag. The slag used may be the normal slag forming on the bath from oxidation of the copper, or it may be a special slag as desired.

It will be understood that where copper is already free from sulphur, it may be charged into furnace 17 without preliminary calcining to eliminate sulphur. However, as the movement through the flue serves to preheat the copper charges, thus increasing the economy of operation, I prefer even in that case to use a furnace of the type of furnace A. It would of course be possible to preliminarily desulphurize and intermediately cool the cathodes before charging them into furnace 17.

Having melted the sulphur-free copper, I next proceed to reduce by carbon any oxygen present, thus avoiding the possibility of reactions with reducing gases which may be dissolved in the copper. No blowing is necessary since the sulphur is already low, and, since no blowing is required, the copper need not be poled.

In order to reduce the cuprous oxide, I pour the metal from the pool 18 of furnace A into furnace B. Furnace B is free from gases of combustion, and is heated electrically or by any other suitable means. In my figure I show electrodes 24 passing through the wall 25 of the reducing furnace or deoxidizing vessel, and sealed, to prevent entrance of air, by collars 26 and 27. The electrodes are connected to a suitable current source, not shown. While I show an electric furnace employing carbon electrodes, I need not restrict myself to this particular type of electric furnace, and any conventional electric furnace, resistance or induction, may be used as my furnace B. Copper from the bath 18 is preferably charged into the inlet opening 28 of furnace B through a closed trough 29 heated by a burner 30. Slag is retained in the furnace 17 by a gate 31.

The furnace B is filled, both above and below the level of the copper, with coke or other suitable carbonaceous material which will not contaminate the copper with hydrogen or water vapor. Coke is a harmless carbonaceous reducing agent which is forced in through the openings 32 and 33 near the top, by means of plungers 32' and 33'. The heating in the furnace is partly due to the electrical resistance of the coke surrounding the electrodes, since the electrodes will not usually be immersed in the bath. The copper bath 34 may be drawn off as desired through the tap opening 35 and the pouring spout 36 at the end of the furnace.

In ordinary operation the level of the pouring spout is slightly above that of the copper bath 34, so that the furnace must be rotated slightly in order to pour from the spout. For convenience in rotation I preferably make my furnace B circular in cross section. For rotating the furnace I provide suitable supporting rollers 37 engaging bands 38, and also a gear driving band 39 engaged by a rack 40 which is moved back and forth by a screw 41 through a non-rotatable nut 42, secured

to the rack 40. A work hole 43 is provided in the top of the furnace.

The tilting mechanism for the furnace may be used to agitate the copper in contact with the carbon, if desired, but I do not consider agitation necessary to accomplish the reduction of cuprous oxide.

The reactions taking place in the reducing furnace during the first stage of reduction are as follows:



Carbon monoxide produced in Reaction (12) will dissolve in the copper until the copper becomes saturated. Carbon dioxide formed from Reaction (13) will also tend to saturate the copper.

The carbon monoxide is not objectionable because it is not produced by the reaction between any remaining cuprous oxide and the reducing gases during solidification, nor does its solubility change markedly during solidification. But I wish to have the copper bath unsaturated with carbon dioxide to allow for the possible formation of carbon dioxide during the cooling period by oxidation of carbon monoxide. Therefore, I continue the contact between the carbon and the copper until all of the cuprous oxide is reduced. When this has taken place the carbon will reduce carbon dioxide as follows:



In order to reduce carbon dioxide to carbon monoxide, I prolong the dioxidation after the cuprous oxide is effectively eliminated. Any substantial excess of carbon monoxide above that required to saturate the bath will pass off at this stage, and the carbon monoxide passing off will protect the copper from contamination with other gases. Thus I will obtain copper substantially free from cuprous oxide and containing practically no dissolved gas other than carbon monoxide.

The carbon monoxide dissolved in the copper has a "buffer" action in protecting the copper from increase in cuprous oxide content. This carbon monoxide, produced by Reaction (14), is formed from carbon dioxide which was formerly dissolved in the copper, so that after Reaction (14) is complete, the carbon dioxide will be removed from the copper, and carbon monoxide produced instead. Notwithstanding that two volumes of carbon monoxide are produced from one volume of carbon dioxide, most of the carbon monoxide resulting from Reaction (14) will remain dissolved in the copper because carbon monoxide is quite soluble in molten copper, while carbon dioxide is only sparingly soluble under the same conditions.

Now, as previously pointed out, it is entirely possible that an effective quantity of oxygen will be introduced into the copper before the copper solidifies, either due to leakage of air into the copper deoxidation furnace or due to contamination with air at the pouring spout or in the mold during casting. By its "buffer" action, the carbon monoxide will care for a slight contamination with oxygen by reaction with the oxygen to form carbon dioxide. The "buffer" action of carbon monoxide is in addition to the ability of carbon monoxide to react with existing cuprous oxide in the supernatant liquid during solidification. Since the copper has been deliberately unsaturated with carbon dioxide, the carbon dioxide resulting from the "buffer" action of carbon monoxide will not oversaturate the copper, and so will not

produce gas cavities. It is of course obvious that protection from oxygen is highly important because the quantity of oxygen which may be cared for by the "buffer" action of the carbon monoxide is limited.

While I have shown one furnace B in Figure 1, it will be evident that I may employ any conventional arrangement, using two or more such furnaces in series to treat the molten copper successively, as shown for slag deoxidation in Lukens and Heuer Patent, No. 1,733,419, granted October 29, 1929.

The reduced copper from furnace B will ordinarily be poured into molds. In Figure 1 I illustrate diagrammatically conventional casting apparatus consisting of a conventional casting wheel having supporting structure 44 and molds 45, adapted to be moved in either direction to a position registering with the pouring spout 36, when 20 copper may be poured through openings 46 into the molds. In order to minimize contact between the air and the oxide-free copper during casting, and decrease the absorption of oxygen, I pour preferably into vertical molds. By this method 25 I eliminate the "set" or oxidized copper surface obtained on horizontal castings. For best results I also surround the stream of pouring copper with a nonoxidizing gas, preferably carbon monoxide, since the copper under ordinary conditions will 30 already be saturated with carbon monoxide, to prevent the absorption of atmospheric gases, especially oxygen. I illustrate at 47 conventional means for surrounding the stream of pouring copper with an atmosphere of carbon monoxide. 35 The molten copper may simply be poured in a chamber containing carbon monoxide.

Thus it will be seen that my process consists of the following steps, desirably in succession: (1) removing sulphur from the cathodes; (2) melting; 40 (3) reducing cuprous oxide; (4) reducing carbon dioxide; (5) casting. The first step might be eliminated if sulphur-free material could be obtained, and of course the sulphur might less desirably be removed after melting. In the preferred form of my invention the elimination of sulphur is accomplished before melting, but this is not essential, especially if the conventional copper melting reverberatory furnace is to be used, since the copper can be charged into such 45 a furnace either continuously or intermittently, with or without preheating, can be melted, blown to remove sulphur if desired, poled to remove part of the oxygen content, deoxidized by treatment in the deoxidation furnace B and cast, preferably with proper protection. The last step, while offering a desirable combination in the practice of my invention, could be dispensed with if it were desired to transfer the copper to a storage furnace, 50 for example.

Independently of the role of cuprous oxide, the presence of hydrogen in the copper bath is undesirable because of its tendency to form gas cavities due to its decrease in solubility during solidification. Green poles previously used to reduce copper oxide of course introduce a large quantity of hydrogen into the bath in the form of hydrocarbons. By avoiding the use of material rich in hydrogen in the deoxidizing furnace, as by 55 employing charcoal or coke, I avoid introducing excessive quantities of hydrogen into the bath.

It will be understood that my invention could be carried out entirely in one furnace, where the calcining, melting, and reducing operations would proceed. This, however, would be slow and less

desirable than the continuous method of operation using two or more furnaces.

It will be evident that the elimination of sulphur is necessary in those cases only where the raw copper material has an excessive sulphur content—which represents the normal condition—; also that the elimination of blowing and poling keeps down the amount of cuprous oxide and carbon dioxide present and avoids the necessity for excessive reduction by carbon to take care of this condition; that the reduction of cuprous oxide and subsequently of carbon dioxide below the saturation point of carbon dioxide is highly essential and is secured most quickly and most effectively by immersion of the carbon within the molten copper bath; and that casting within vertical molds reduces the subsequent air contamination with its increase of cuprous oxide and carbon dioxide within the solid copper.

By my statements that the atmosphere surrounding the copper during deoxidation will contain so little carbon dioxide and hydrogen as not to harmfully affect the copper, I do not mean to imply that any substantial percentage of carbon dioxide or hydrogen is present, as the atmosphere will preferably contain no substantial percentage of carbon dioxide and hydrogen. I merely mean that the quantity of carbon dioxide and hydrogen, if any be present, will not be sufficient to affect the copper harmfully.

When I refer herein to complete removal of cuprous oxide present in the copper, to complete deoxidation of the copper, or to any similar thought, I of course wish to indicate that removal of cuprous oxide is complete according to the tests commonly used by the copper metallurgist at the time of filing this application for patent, such as microscopic examination, so that no distinct phase of cuprous oxide is visible in the solid copper. I do not mean to indicate that cuprous oxide which may remain in solid solution 40 in the solid copper, as determined by methods developed subsequently to my date of filing this application, is necessarily absent.

It will be evident that, where reference is made in the specification and claims to a casting or to casting, it is intended to designate a commercial product having the properties such as malleability and ductility of a commercial casting, and its process of manufacture, and not merely a laboratory or museum specimen and its process of manufacture.

In view of my invention and disclosure variations and modifications to meet individual whim or particular need will doubtless become evident to others skilled in the art, to obtain part or all 55 of the benefits of my invention without copying the structure shown, and I, therefore, claim all such in so far as they fall within the reasonable spirit and scope of my invention.

Having thus described my invention, what I 60 claim as new and desire to secure by Letters Patent is:—

1. In the art of preparing copper for making castings substantially free from cuprous oxide and gas cavities, the process which consists in desulphurizing copper cathodes in the solid state, in melting them free from contact with sulphur, the melt produced containing cuprous oxide, in reducing dissolved cuprous oxide in the molten copper bath by large surface contact with carbon in an atmosphere having insufficient carbon dioxide and hydrogen to harmfully affect the copper and in prolonging the reduction until the harmful content of carbon dioxide in the copper is removed.

2. In the art of preparing copper for making castings substantially free from cuprous oxide and gas cavities, the process which consists in removing sulphur from the solid copper charges to avoid the necessity of blowing and consequent boiling, in melting the charges free from contact with sulphur, the molten copper containing cuprous oxide and carbon monoxide, and in unsaturating the metal from carbon dioxide in order that it may take up carbon dioxide during solidification without becoming over-saturated with carbon dioxide.

3. The process of purifying copper cathodes, which consists in heating cathodes in the presence of hydrogen to volatilize sulphur as hydrogen sulphide, melting the cathodes free from contamination with sulphur, reducing substantially all of the cuprous oxide present in the copper by contact with carbon in an atmosphere having insufficient carbon dioxide and hydrogen to harmfully affect the copper and in prolonging the reduction until the content of oxides of carbon in the copper is harmless.

4. The process of making copper castings substantially free from cuprous oxide and objectionable gas cavities, which consists in reducing sulphur by heating copper cathodes in the presence of hydrogen, melting the cathodes under oxidizing conditions to eliminate dissolved hydrogen while avoiding contamination with sulphur, substantially completely reducing cuprous oxide present in the copper and casting the purified material.

5. The process of treating copper, which consists in roasting solid copper cathodes to eliminate sulphur, in melting the cathodes free from contamination with sulphur and in treating the molten copper with carbon throughout the body of the copper for a duration sufficient to render the remainder of the oxides of carbon in the copper harmless, in an atmosphere having so little carbon dioxide and hydrogen as not to harmfully affect the copper.

6. In the art of making copper castings substantially free from cuprous oxide and gas cavities, the process which consists in melting substantially sulphur-free copper in a melting furnace under conditions which produce oxygen-bearing molten copper, in protecting the copper from contamination with substances rich in hydrogen subsequent to melting, in transferring the molten copper to a deoxidizing vessel, in treating the molten copper in the deoxidizing vessel with carbon submerged throughout the body of the molten copper in an atmosphere substantially free from hydrogen for a time sufficient to reduce carbon dioxide, in maintaining dissolved carbon monoxide in the molten copper, in transferring the molten copper from the deoxidizing vessel to the point of casting and in subsequently cooling the molten copper to solidify it while free from admixture with carbon throughout the molten copper.

7. The process of treating copper, which consists in roasting solid copper charges to eliminate sulphur, in melting the charges free from contamination with sulphur, in treating the molten copper with carbon throughout the body of the copper, in an atmosphere having insufficient carbon dioxide and hydrogen to harmfully affect the copper, in prolonging the reduction until the harmful content of gas in the copper is removed, in casting the copper and in protecting the copper from air during casting by a harmless gas having a sufficiently low partial pressure of oxy-

gen so as not to contaminate the copper with oxygen.

8. In the art of producing copper castings substantially free from gas cavities, using a fuel-fired furnace and an electric furnace, the process which consists in preparing oxygen-bearing molten copper in the fuel-fired furnace, in transferring the molten copper to the electric furnace, in eliminating cuprous oxide from the molten copper by carbon reduction in the electric furnace, in continuing the reduction to unsaturate the molten copper with carbon dioxide, in casting the copper and in protecting the copper from excessive contact with air during casting.

9. The process of preparing copper castings practically free from gas cavities and cuprous oxide, which consists in treating molten copper with carbon submerged throughout the copper to reduce the cuprous oxide until too little cuprous oxide remains in the bath to react with impurities in the copper during solidification and liberate carbon dioxide or water vapor from the copper, in reducing carbon dioxide in the molten copper to carbon monoxide, in distributing carbon monoxide in the molten copper, in separating the molten copper from the carbon, in casting the copper in pure condition and in protecting the copper from contact with air during casting.

10. The process of purifying molten copper and of producing the copper in solid form, which consists in reducing dissolved carbon dioxide, present in the molten copper by reason of the reaction between cuprous oxide and carbon monoxide, to carbon monoxide by contact with carbon maintained submerged throughout the molten copper, in maintaining carbon monoxide in the molten copper, in separating the molten copper from the carbon and in withdrawing and solidifying the copper in pure condition free from excessive contamination with air.

11. The process of producing copper castings free from excessive gas cavities, which consists in exposing the molten copper to a large surface of carbon submerged throughout the copper free from contamination of substances rich in hydrogen preliminary to casting, in separating the molten copper from the carbon, in casting the copper in pure condition and in protecting the copper from air during casting by surrounding the copper with carbon monoxide free from contamination with substances which will cause the liberation of carbon dioxide, hydrogen or steam in the solidifying copper.

12. The process of producing copper castings free from excessive gas cavities, which consists in deoxidizing the copper, in dissolving carbon monoxide in the copper, in carrying the deoxidation to an extent such that carbon dioxide is removed until the quantity of carbon dioxide left is not objectionable during casting, in casting the copper in pure condition and in protecting the copper from oxidizing gases, during casting, by carbon monoxide free from substances which will cause the liberation of carbon dioxide, hydrogen or steam in the solidifying copper.

13. In the art of producing copper castings free from objectionable gas cavities, the process which consists in preheating solid copper charges, in melting the charges by fuel combustion while exposed to a bath of molten copper, in transferring the molten copper to a deoxidizing vessel, in deoxidizing the molten copper by the action of carbon monoxide free from substances which will cause hydrogen or steam to be liberated in the copper during solidification, in transferring

- the molten copper from the deoxidizing vessel to the point of casting and in casting the copper in pure condition while blanketing it with a gas having a predominantly reducing component of
- 5 carbon monoxide and having a sufficiently low partial pressure of oxygen so as not to contaminate the copper with oxygen or its compounds other than carbon monoxide.
14. In the art of producing copper castings 10 free from cuprous oxide and objectionable gas cavities, the process which consists in preheating solid copper charges, thereby producing oxygen-bearing molten copper, in melting the charges, in deoxidizing the molten copper and removing 15 sufficient of the carbon dioxide in the copper to render the remainder harmless, by carbon in a confined space in an atmosphere low in carbon dioxide and hydrogen and in casting the copper in pure condition while protecting the molten 20 copper from excessive contact with air during casting.
15. In the art of producing copper castings substantially free from objectionable gas cavities, using a fuel-fired melting furnace and a deoxidation furnace, the process which consists in preparing oxygen-bearing molten copper in the fuel-fired furnace, in transferring the molten copper to the deoxidation furnace, removing from the molten copper substantially all of the 25 cuprous oxide and sufficient of the gas in the copper to render the remainder harmless by carbon reduction in the deoxidation furnace in an atmosphere having insufficient carbon dioxide and hydrogen to harmfully affect the copper, in 30 casting the copper and in protecting the copper from excessive contact with air during casting.
16. The process of purifying molten copper to substantially remove its content of cuprous oxide and make solid copper of high density, which 40 consists in treating molten copper containing cuprous oxide with carbon in a confined space free from contamination with substances which will cause the liberation of carbon dioxide, hydrogen or steam during solidification of the copper, 45 thereby forming carbon monoxide and taking out some cuprous oxide, in treating the molten copper with the carbon monoxide, thereby distributing carbon dioxide in the molten copper and taking out more cuprous oxide, in reducing carbon dioxide in the molten copper to carbon monoxide by contact with the carbon, in maintaining carbon monoxide in the molten copper and in casting 50 the copper in pure condition while blanketing it with carbon monoxide free from substances which 55 cause the liberation of carbon dioxide, hydrogen or steam in the solidifying copper.
17. The method of treating copper to make castings free from cuprous oxide and objectionable gas cavities, which consists in melting the 60 copper while in contact with products of fuel combustion, and in subsequently removing from the molten copper the cuprous oxide and sufficient of its content of dissolved gas to render the remainder harmless by exposing the copper in 65 molten condition to contact with carbon in the absence of contamination with air and with gases of combustion from hydrocarbon fuel.
18. The method of treating copper to make castings free from objectionable gas cavities, 70 which consists in melting the copper by fuel combustion, in oxidizing the copper to remove sulphur, in completely deoxidizing the cuprous oxide present in the molten copper by carbon while protecting the copper from contamination with air and the harmful gaseous products of the fuel
- combustion, in casting the copper and in shielding the copper during casting from air, oxidizing gaseous products of fuel combustion and hydrogen.
19. In the art of producing copper castings substantially free from gas cavities, the process which consists in substantially eliminating the cuprous oxide content of oxygen-bearing molten copper by reduction with carbon in an atmosphere having insufficient carbon dioxide and 10 hydrogen to harmfully affect the copper, in prolonging the reduction until the harmful content of carbon dioxide is reduced to carbon monoxide, in maintaining carbon monoxide in the molten copper, in separating the molten copper from the 15 carbon and in casting the copper in pure condition free from excessive contact with air.
20. In the art of producing copper castings substantially free from gas cavities, using a fuel-fired melting furnace and an auxiliary deoxidizing furnace, the process which consists in preparing oxygen-bearing molten copper in the fuel-fired melting furnace, in transferring the copper to the auxiliary deoxidizing furnace, in deoxidizing the molten copper by carbon reduction in the 25 deoxidizing furnace in an atmosphere containing so little carbon dioxide and hydrogen as not to harmfully affect the copper, in casting the copper and in protecting the copper from excessive contact with air during casting by a noncontaminating 30 reducing gas.
21. In the art of producing copper in refined form, the process which consists in melting the copper in a fuel-fired furnace, thereby making oxygen-bearing molten copper, in transferring the molten copper to a deoxidizing furnace, in deoxidizing the molten copper completely in the deoxidizing furnace by intimate contact with carbon in the absence of air and gases resulting from the combustion of hydrocarbon fuel, thereby making completely deoxidized molten copper and in casting the molten copper while protecting it from air by a reducing gas containing a 35 substantial concentration of carbon monoxide.
22. The process of treating copper to produce 45 castings free from a distinct phase of cuprous oxide and objectionable gas cavities, which consists in preheating solid copper charges, in melting the copper by fuel combustion, while surrounded by molten copper, to produce a copper 50 melt containing cuprous oxide, in completely deoxidizing the cuprous oxide present in the molten copper by carbon in an atmosphere having so little carbon dioxide and hydrogen as not to harmfully affect the copper, in casting the copper 55 and in protecting the copper during casting from excessive contact with air by a gas having a predominantly reducing component of carbon monoxide and having a sufficiently low partial pressure of oxygen so as not to contaminate the copper with oxygen or its compounds other than carbon monoxide.
23. The process of treating copper to produce 60 castings free from a distinct phase of cuprous oxide and objectionable gas cavities, which consists in preheating solid copper charges, in melting the copper, surrounded by molten copper, by fuel combustion to produce a copper melt containing cuprous oxide, in completely deoxidizing the cuprous oxide present in the molten copper 65 by carbon and prolonging the deoxidation with carbon for a time sufficient to render the remainder of the oxides of carbon harmless, under 70 conditions of freedom from fuel combustion in an atmosphere having so little carbon dioxide 75

- and hydrogen as not to harmfully affect the copper, in casting the copper and in protecting the copper during casting from excessive contact with air.
- 5 24. The method of treating copper to produce castings free from cuprous oxide and objectionable gas cavities, which consists in melting the copper by fuel combustion in which the gases of combustion are in contact with the molten copper to produce a molten bath containing cuprous oxide and in removing from the copper cuprous oxide and prolonging the deoxidation for a time sufficient to render the remainder of the oxides of carbon harmless, by maintaining the copper in molten condition in contact with carbon in an atmosphere having so little carbon dioxide and hydrogen as not to harmfully affect the copper.
- 10 25. The process of purifying copper, which consists in preparing oxygen-bearing molten copper under fuel-fired conditions in which the molten copper is exposed to the products of fuel combustion, in exposing the molten copper in a confined space to contact with carbon while protecting the copper from air and products of fuel combustion, in agitating the molten copper while it is in contact with the carbon for a time sufficient to completely deoxidize the copper and effect removal of harmful gas from the copper, in transferring the molten copper from the confined space to the point of casting and in subsequently cooling the molten copper to solidify it.
- 15 26. The process of producing copper castings, which consists in removing cuprous oxide from molten copper by contact with carbon, in continuing the reduction by carbon to reduce carbon dioxide to carbon monoxide, in agitating the copper while it is in contact with the carbon and in casting the copper while surrounding it with a gas which is harmless to the copper.
- 20 27. The process of deoxidizing molten copper, which consists in melting the copper by fuel combustion in which the gases of combustion are in contact with the molten copper, in exposing it to contact with carbon in a confined space to remove cuprous oxide, in continuing the contact with carbon after the removal of cuprous oxide to change carbon dioxide to carbon monoxide and in producing forced agitation of the molten copper while it is in contact with the carbon.
- 25 28. The method of refining metals which readily oxidize upon exposure to air in their molten state, which comprises subjecting the metal to an oxidizing reaction to remove sulphur, melting the metal with fuel heating flames, subjecting the metal in molten condition to a complete reaction with a harmless carbonaceous reducing agent to remove substantially all of the metallic oxides while keeping the metal protected from the air and the contaminating products of combustion of fuel heating flames, and pouring the metal while protecting it from the air and the contaminating products of combustion of fuel heating flames.
- 30 29. The method of refining copper, which comprises subjecting the metal to an oxidizing reaction to remove sulphur, melting the metal in a fuel fired reverberatory furnace, subjecting the oxidized metal in molten condition to a complete reaction with a harmless carbonaceous reducing agent to remove substantially all of the metallic oxides while fully protecting the metal from the atmospheric air and the contaminating products of combustion of fuel heating flames, and pouring the metal while protecting it from the air and the contaminating products of combustion of fuel heating flames.
- 35 30. The method of refining copper which comprises, melting the copper in a fuel-fired furnace which tends to oxidize the metal, transferring the metal to a treating vessel and there subjecting it in molten condition to a complete reaction with a harmless carbonaceous reducing agent by bringing all of the metal into thorough contact with the reducing agent while keeping the metal protected from the air and the contaminating products of combustion of fuel heating flames to perform a complete reducing action on the metal, and pouring the oxygen-free copper while protecting it from air by a gas composed principally as to active constituent of carbon monoxide.
- 40 31. The method of refining copper, which comprises, melting the copper in a fuel fired reverberatory furnace, oxidizing the copper to remove sulphur, subjecting the copper in molten condition to a complete reaction with a harmless carbonaceous reducing agent by bringing all of the metal into thorough and intimate contact with the reducing agent while keeping the metal protected from the air and the contaminating products of combustion of fuel heating flames to remove substantially all of the metallic oxides, and casting the metal while protecting it from oxidizing influences and the contaminating products of combustion of fuel heating flames.
- 45 32. In the art of making castings free from cuprous oxide and of high density, the process which consists in preheating solid copper charges, in subsequently carrying the charges to a melting furnace and there melting the charges under conditions which produce oxygen-bearing molten copper, in agitating the molten copper in a confined space and a noncontaminating atmosphere in direct contact with carbon for a sufficient duration to remove enough carbon dioxide to render the remainder harmless to the copper and in cooling the molten copper, in a mold separate from the confined space, to solidify the copper.
- 50 33. In the art of preparing copper for making castings free from cuprous oxide and of high density, the process which consists in preheating solid copper charges, in melting the charges while in contact with a bath of molten copper under conditions which produce oxygen-bearing molten copper and in treating the molten copper with carbon for a duration sufficient to render the remainder of the carbon dioxide in the copper harmless, to deoxidize the molten copper in a confined space protected from substances which will cause gas cavities due to liberation of carbon dioxide, hydrogen or steam in the copper during solidification.
- 55 34. In the art of making copper castings substantially free from cuprous oxide and excessive gas cavities, the process which consists in treating molten copper containing cuprous oxide with carbon monoxide, thereby taking out cuprous oxide and distributing carbon dioxide in the molten copper, in reducing the carbon dioxide so formed by carbon in contact with the molten copper in a confined space free from substances which cause the liberation of hydrogen or steam in the solidifying copper, in maintaining carbon monoxide in the molten copper, in transferring the molten copper from the confined space to the point of casting and in subsequently cooling the molten copper to solidify it.
- 60 35. The process of preparing copper castings practically free from gas cavities and cuprous oxide, starting with electrolytically refined copper, which consists in melting the copper in a fuel-fired melting furnace having the gases of

5 combustion in contact with the molten copper, under melting conditions which produce oxygen-bearing molten copper, in transferring the oxygen-bearing molten copper to a separate de-  
 10 oxidizing furnace, in there treating the molten copper with carbon until the molten copper is practically completely deoxidized and too little oxygen remains in the molten copper to react with impurities in the copper during solidifica-  
 15 tion and form gas cavities due to liberation of carbon dioxide or water vapor from the copper, in separating the molten copper from the carbon and in casting the copper under conditions which maintain a harmless oxygen content in the solidifying copper due to avoidance of excessive contact with atmospheric gases during casting.  
 20 36. The process of preparing copper castings practically free from gas cavities and cuprous oxide, starting with electrolytically refined copper, which consists in melting the copper in a fuel-fired melting furnace having the gases of combustion in contact with the molten copper, under melting conditions which produce oxygen-bearing molten copper, in transferring the oxygen-bearing molten copper to a separate electrically heated deoxidizing furnace, in there treating the molten copper with carbon until the molten copper is practically completely deoxidized and too little oxygen remains in the molten copper  
 25 to react with impurities in the copper during  
 30

solidification and form gas cavities due to libera-  
 5 tion of carbon dioxide or water vapor from the copper, in separating the molten copper from the carbon and in casting the copper under conditions which maintain a harmless oxygen content in the solidifying copper due to avoidance of excessive contact with atmospheric gases during casting.

37. The process of preparing copper castings practically free from gas cavities and cuprous oxide, which consists in preheating copper masses 10 in a preheating furnace, in transferring the pre-heated copper masses to a melting furnace, in melting the copper masses in a fuel-fired melting furnace under conditions which produce oxygen-bearing molten copper, in transferring the oxygen-bearing molten copper to a deoxidizing furnace, in there treating the molten copper with carbon until the molten copper is practically completely deoxidized and too little oxygen remains in the molten copper to react with impurities in the copper during solidification and form gas cavities due to liberation of carbon dioxide or water vapor from the copper, in dissolving carbon monoxide in the molten copper, in separating the molten copper from the carbon and in casting the copper under conditions which maintain a harmless oxygen content in the solidifying copper due to avoidance of excessive contact with atmospheric gases during casting.

RUSSELL P. HEUER. 30

### Certificate of Correction

Patent No. 2,060,078.

November 10, 1936.

RUSSELL P. HEUER

It is hereby certified that error appears in the printed specification of the above numbered patent requiring correction as follows: Page 2, first column, line 4, in the equation, for "CuO" read  $Cu_2O$ ; and that the said Letters Patent should be read with this correction therein that the same may conform to the record of the case in the Patent Office.

Signed and sealed this 23rd day of February, A. D. 1937.

[SEAL]

HENRY VAN ARSDALE,  
*Acting Commissioner of Patents.*



**Certificate of Correction**

Patent No. 2,060,073.

November 10, 1936.

**RUSSELL P. HEUER**

It is hereby certified that error appears in the printed specification of the above numbered patent requiring correction as follows: Page 2, first column, line 4, in the equation, for "CuO" read  $Cu_2O$ ; and that the said Letters Patent should be read with this correction therein that the same may conform to the record of the case in the Patent Office.

Signed and sealed this 23rd day of February, A. D. 1937.

[SEAL]

**HENRY VAN ARSDALE,**  
*Acting Commissioner of Patents.*